

## UNITED STATES PATENT OFFICE

JOHN A. SUCCOP, OF PITTSBURGH, PENNSYLVANIA, ASSIGNOR TO HEPPENSTALL COMPANY, OF PITTSBURGH, PENNSYLVANIA, A CORPORATION OF PENNSYLVANIA

## ALLOY STEEL

No Drawing. Application filed June 12, 1930. Serial No. 460,791.

This invention relates to alloy steels and articles made therefrom, and especially to steels for the production of edged articles.

A major object of the invention is to provide alloy steels embodying a desirable combination of physical properties, which do not require abnormal heat treatments, which when heat treated possess very high ductility and cohesive strength, develop high hardness and resistance to abrasion, are relatively non-corrodible and non-tarnishing, are especially adapted for the production of keen edged articles capable of withstanding rapid edge destruction, and which are readily made and fabricated.

It is among other objects of the invention to provide edged articles, and particularly razor blades, which possess keen cutting edges having long useful life, and which are markedly stable surfaced.

The alloy steels provided by this invention contain carbon and chromium in amounts adapted to confer useful physical properties and surface stability, together with nickel, vanadium and molybdenum as characterizing elements in amounts to intensify and stabilize the effects of the carbon and chromium, and they also contain constituents usual in alloy steels, such as manganese and silicon.

In its broader aspects the invention contemplates steels containing from about 0.5 to 2.50 per cent of carbon, about 5.0 to 20.0 per cent of chromium, about 0.10 to 1.75 per cent of manganese, about 0.05 to 2.0 per cent of molybdenum, about 2.5 to 3.5 per cent of nickel, about 0.10 to 2.0 per cent of silicon, and about 0.05 to 1.5 per cent of vanadium, the balance of the alloy being iron with the impurities incidental to commercial steel manufacture. In these alloys phosphorous and sulfur are preferably kept as low as possible, most suitably below about 0.03 per cent.

In its preferred embodiment the invention contemplates the use of steels having a com-

position falling substantially within the following range:

|            | Per cent     |
|------------|--------------|
| Carbon     | 0.70 to 1.75 |
| Chromium   | 10.0 to 16.0 |
| Manganese  | 0.15 to 0.30 |
| Molybdenum | 0.40 to 1.50 |
| Nickel     | 0.80 to 2.00 |
| Silicon    | 0.20 to 0.45 |
| Vanadium   | 0.30 to 1.00 |
| Iron       | Balance      |

Within these ranges of composition particularly desirable results are obtained by varying the contents of carbon, molybdenum and nickel with respect to chromium, in a manner hereinafter set forth.

If desired for particular purposes the alloys may also contain other constituents such as those now commonly added to special alloy steels, for example uranium, titanium, tungsten, or cobalt, the content of such added alloy elements, either individually or in total, preferably not exceeding about 3 per cent.

Steels made from compositions within these ranges possess a particularly valuable combination of structural, physical, and working, or fabricating, properties. For example, they may be heat treated over wide ranges of temperatures. My tests show that these alloys may be quenched at temperatures between about 1700 to 1900° F., and that they may be tempered over a considerable range of temperature, without adversely affecting their physical properties. On the contrary, when quenched or drawn over these extremes, more desirable physical properties are obtained, and carbide segregation is less pronounced, than is the case with tool steels generally. In general it is preferred to preheat the steels followed by relatively rapid heating to a quenching temperature of about 1750 to 1825° F., and then quench in oil.

The steels provided by this invention are

further characterized by high hardness and tensile strength combined with great ductility for a given hardness. They therefore possess high elastic capacity which permits severe service distortion without taking permanent set, and they also possess high resistance to abrasion.

These features may be understood from one set of tests, in which a high quality 10 Swedish tool steel containing 1.0 per cent of carbon and 0.4 per cent of manganese, was compared with two steels embodying this invention, whose composition was approximately as follows:

|    |                 | Steel A  | Steel B  |
|----|-----------------|----------|----------|
|    |                 | Per cent | Per cent |
| 15 | Carbon.....     | 0.70     | 1.75     |
| 20 | Chromium.....   | 10.0     | 16.0     |
|    | Manganese.....  | 0.25     | 0.25     |
|    | Molybdenum..... | 0.40     | 1.50     |
|    | Nickel.....     | 0.80     | 2.0      |
|    | Silicon.....    | 0.35     | 0.35     |
|    | Vanadium.....   | 0.30     | 1.00     |

Samples of these three steels were heat treated simultaneously, by quenching from about 1750-1800° F., followed by drawing at various temperatures, after which physical tests were made. The results obtained are shown in the following table:

|    |                         | Tensile strength<br>lbs. per sq.<br>in. | Elongation<br>per cent in 2" | Hardness<br>Brinell<br>No. |
|----|-------------------------|-----------------------------------------|------------------------------|----------------------------|
| 35 | Swedish steel:          |                                         |                              |                            |
|    | Tempered at 560° F..... | 254,000                                 | 4.0                          | 480                        |
|    | Tempered at 750° F..... | 200,000                                 | 7.0                          | 400                        |
| 40 | Steel A:                |                                         |                              |                            |
|    | Tempered at 560° F..... | 290,500                                 | 2.0                          | 600                        |
|    | Tempered at 750° F..... | 280,000                                 | 2.5                          | 600                        |
|    | Steel B:                |                                         |                              |                            |
|    | Tempered at 560° F..... | 325,000                                 | 1.8                          | 600                        |
|    | Tempered at 750° F..... | 305,000                                 | 2.0                          | 600                        |

These data show that much greater tensile strengths are obtained, with concomitant greater hardness from my new steels, and 45 that drawing over this range does not apparently affect the hardness, whereas the hardness of the Swedish steel decreases substantially. Further tests showing these properties follow:

|    |                          | Tensile strength,<br>lbs. per<br>sq. in. | Elonga-<br>tion, per<br>cent in<br>2" | Hardness<br>Brinell<br>No. |
|----|--------------------------|------------------------------------------|---------------------------------------|----------------------------|
| 55 | Steel A:                 |                                          |                                       |                            |
|    | Tempered at 930° F.....  | 271,000                                  | 3.5                                   | 589                        |
|    | Tempered at 1100° F..... | 225,000                                  | 6.8                                   | 555                        |
|    | Steel B:                 |                                          |                                       |                            |
|    | Tempered at 930° F.....  | 300,000                                  | 2.7                                   | 600                        |
|    | Tempered at 1100° F..... | 270,000                                  | 4.7                                   | 587                        |

60 My present belief is that the remarkable properties of these alloys result from the use of a balanced composition in which the various constituents coact to produce a structure in which coalescence of excess carbides into 65 a network structure is prevented. It appears

the composition of the steels is such that proper heat treatment of these alloys produces a structure comprising minute carbide particles embedded in a matrix composed principally of a solid solution or solid solutions of 70 nickel, molybdenum and vanadium in iron, from which the carbide is not readily rejected, this being a martensitic structure. The matrix provides the substantial toughness, fibre strength, and ductility which is characteristic of the alloys provided by the invention, while hardness results from the dispersion in the matrix of the exceedingly hard particles of carbide, hardness retention being favored by the minimized tendency toward 80 carbide rejection.

Whether or not the foregoing belief as to the structural composition of the new steels is correct, it is a fact that the new steels develop a refined structure possessing 85 a combination of very high ductility, fibre or cohesive strength, and hardness which adapts them especially for the production of keen edged articles in which these properties manifest themselves by resistance to edge destruction. Although flint hardness is not always a prerequisite in the production of 90 satisfactory cutting edges, it is possible to obtain with these alloys a Brinell hardness number of over 600, a hardness on the Rockwell C scale of over 65, or scleroscope of more than 85. Furthermore, after heat treatment, and particularly upon being highly polished, articles made from them possess substantial 95 surface stability, evidenced by resistance to 100 corrosion as by etching reagents, tarnishing and atmospheric oxidation.

These desirable properties are apparently due to a balance between the constituents, and in varying the composition of the alloys 105 within the ranges given, the most suitable results are obtained by controlling the contents of carbon, molybdenum and nickel in accordance with variations in the chromium content. More specifically my tests have shown 110 that to obtain the best results, within the preferred ranges at least, as the chromium is increased from 10 to 16 per cent the molybdenum and nickel contents vary according to practically straight line ratios between 0.4 115 and 1.5 per cent, and between 0.8 and 2.0 per cent respectively. Also, as chromium is increased within the same limits, carbon is preferably increased from 0.7 to 1.75 per cent, the increments being greater for the 120 lower ranges of chromium, and becoming smaller toward the upper limits. Stated in other words, within the ranges given molybdenum and nickel vary in substantially direct proportion to the chromium content, while the carbon content variably increases at a diminishing rate as the chromium content increases.

The combination of physical properties 125 capable of being developed in these alloys 130

confers the further advantage that it makes possible the production of thin sections having intricate designs, such as those of the recent types of safety razor blades, in which the article, because of its high ductility, resists breakage either in manufacture or in use. For example, a wafer type razor blade having a thickness of 0.006 inch held at the ends can be bent repeatedly to an angle of forty-five degrees without breaking or taking a permanent set.

The properties of these alloys render them particularly suitable for the production of razor blades, not only because their cutting edges possess unusual resistance to abrasion and edge destruction, but also for the reason that rusting and electrolytic action, for example between the blade and its holder, is reduced to such a point that the necessity of thoroughly drying parts before storage is substantially eliminated. Such blades therefore possess materially longer life than those heretofore commercially available.

In the production of razor blades it is preferred to use alloys of about the following composition:

|            | Per cent      |
|------------|---------------|
| Carbon     | 0.70 to 0.75  |
| Chromium   | 10.0 to 12.00 |
| Manganese  | 0.15 to 0.30  |
| Molybdenum | 0.40 to 0.50  |
| Nickel     | 0.80 to 1.00  |
| Silicon    | 0.20 to 0.45  |
| Vanadium   | 0.35 to 0.45  |
| Iron       | Balance       |

The unusually great ability of articles made from these alloys to retain a cutting edge may be shown best by tests made with safety razor blades made therefrom. One hundred sets of razor blades each comprising a blade made from an alloy of the preferred composition just given (Blade A), a blade made from the best razor blade steel heretofore available (Blade B), and a standard commercial blade (Blade C), were distributed for the purpose of obtaining an unbiased and disinterested test, the results being reported in number of satisfactory shaves had from each blade. A tabulation of the results follows:

|                    | Number of shaves |         |         |
|--------------------|------------------|---------|---------|
|                    | Blade C          | Blade B | Blade A |
| Average            | 3                | 11      | 24      |
| Highest individual | 7                | 24      | 50      |

These results show the marked superiority of blades made from my alloys. They show that on an average such blades retain their edge twice as long as those made from the best known razor steel, and eight times longer than those of the average commercially obtainable blade. Similar results were obtained with shear knives used to cut tin-plate, where knives made from these alloys possessed a useful life of weeks, while the

best available knives have a life of but a few days.

The production and fabrication of these alloys presents no unusual difficulties, the practice being that normal to commercial alloy products. In addition to the wide range of heat treating temperatures referred to, these alloys also possess the property of being resistant to prolonged soaking at or near the quenching temperature.

According to the provisions of the patent statutes, I have explained the principle and mode of operation of my invention, and have specifically described what I now consider to represent its best embodiment. However, I desire to have it understood that, within the scope of the appended claims, the invention may be practiced otherwise than as specifically described.

I claim:

1. An alloy steel for the production of abrasion-resistant edged articles and having a martensitic structure, the alloy consisting of from about 0.5 to 2.0 per cent of carbon, from about 5.0 to 20.0 per cent of chromium, from about 0.1 to 1.75 per cent of manganese, from about 0.1 to 2.0 per cent of molybdenum, from about 0.25 to 3.5 per cent of nickel, from about 0.1 to 2.0 per cent of silicon, and from about 0.1 to 1.5 per cent of vanadium, the remainder being iron except for elements present as impurities and in amounts insufficient to materially alter the physical and abrasion-resistant properties of said alloy, the elements of the alloy being balanced by varying between the stated limits the molybdenum and nickel contents in substantially direct proportion to changes in chromium content, and by variably increasing the carbon content at a diminishing rate as the chromium is increased.

2. An alloy steel for the production of abrasion-resistant edged articles and having a martensitic structure, the alloy consisting of from about 0.6 to 1.75 per cent of carbon, from about 10.0 to 16.0 per cent of chromium, from about 0.1 to 0.75 per cent of manganese, from about 0.4 to 1.5 per cent of molybdenum, from about 0.8 to 2.0 per cent of nickel, from about 0.1 to 0.75 per cent of silicon, and from about 0.3 to 1.0 per cent of vanadium, the remainder being iron except for elements present as impurities and in amounts insufficient to materially alter the physical and abrasion-resistant properties of said alloy, the elements of the alloy being balanced by varying between the stated limits the molybdenum and nickel contents in substantially direct proportion to changes in chromium content, and by variably increasing the carbon content at a diminishing rate as the chromium is increased.

In testimony whereof, I sign my name.  
JOHN A. SUCCOP.